

O. FALKENWALDE,

PROCESS OF RENDERING MEXICAN FLUX AND CRUDE OILS AVAILABLE AS A FUEL,  
APPLICATION FILED JULY 17, 1914.

1,177,405.

Patented Mar. 28, 1916.



Witnesses

R. J. Jones  
R. H. Meyer.

Inventor

O. Falkenwalde

By *O. Falkenwalde* Attorney

# UNITED STATES PATENT OFFICE.

OSCAR FALKENWALDE, OF BALTIMORE, MARYLAND.

## PROCESS OF RENDERING MEXICAN FLUX AND CRUDE OILS AVAILABLE AS A FUEL.

1,177,405.

Specification of Letters Patent. Patented Mar. 28, 1916.

Application filed July 17, 1914. Serial No. 851,665.

*To all whom it may concern:*

Be it known that I, OSCAR FALKENWALDE, a citizen of the United States, residing at Baltimore, in the State of Maryland, have 5 invented certain new and useful Improvements in Processes of Rendering Mexican Flux and Crude Oils Available as a Fuel; and I do hereby declare the following to be a full, clear, and exact description of the 10 invention, such as will enable others skilled in the art to which it appertains to make and use the same.

This invention relates to processes for rendering Mexican flux and crude oils available as a fuel. Mexican flux or crude oil has not been heretofore regarded as a desirable fuel, for various reasons, but has been used to some extent when mixed with other domestic oils to render the crude oil 15 more fluid. When thus adulterated the product is called Mexican fuel oil. Analysis of the Mexican flux or crude oil shows that it contains naphtha, illuminatory oil, lubricating oil, tar and residuum in varying proportions.

In carrying out my invention, I mix a certain quantity of hot water at a temperature from one hundred and fifty to two hundred and ten degrees Fahrenheit with 20 the Mexican flux or crude oil and feed the water and flux or crude oil to a point to be united and utilized as a fuel immediately after the mixing operation. The compound thus formed burns freely and does not 25 blacken or clog the burner, and owing to its inexpensive character this fuel is very desirable for many purposes.

The relative proportions of the various ingredients of the flux or crude oil is approximately given as follows:

|                  |       |
|------------------|-------|
| Naphtha          | 10.0% |
| Illuminatory oil | 60.0% |
| Lubricating oil  | 15.5% |
| Tar and residuum | 14.5% |

The chemical characteristics of the Mexi-

can flux may be briefly referred to as follows:

|                               |            |    |
|-------------------------------|------------|----|
| Specific gravity at 60° F.    | 0.9854.    | 50 |
| Baumé gravity                 | 12.1.      |    |
| Pound per gallon at 60° F.    | 8.209.     |    |
| Flash point, open cup         | 171° F.    |    |
| Flash point, closed cup       | 75° F.     |    |
| Fire test                     | 252° F.    |    |
| Specific viscosity            | 154/50° C. | 55 |
| Fixed carbon                  | 9.00.      |    |
| Cold test                     | 40° F.     |    |
| B. T. U. per pound            | 18,088.    |    |
| B. T. U. per gallon at 60° F. | 148,484.   | 60 |

The relative proportions of water and flux are approximately: water, 1 part, and Mexican flux, 2 parts.

The figure of the drawing shows an apparatus for performing the process.

The water is usually fed through a needle valve structure A, into and through a tube B from out of which tube it passes into the heating chamber C, traveling through the heating chamber C, and a pipe connection 70 D, into a mixing chamber E, where it is mixed with the Mexican flux or crude oil residue. The Mexican flux or crude oil residue is fed into the mixing chamber E through a needle valve structure F, by the 75 regulation of which the quantity of Mexican flux or oil residue entering the mixing chamber is regulated. The emulsion, which is formed of the heated water and Mexican flux or crude oil residue, passes out of the 80 mixing chamber E, through a burner G for burning. The burner G is positioned directly beneath the water heating compartment C, so that the burning of the emulsion will heat the water within the chamber C 85 to the desired temperature. The water heating compartment C has a pair of tubes H extending upwardly therein, which tubes communicate with the exterior of the burner and interior of the water heating chamber. 90 The overflow tubes H are provided for permitting of the escape of overflow of steam

from the water heating chamber C and also the overflow of water, when the pressure within the chamber exceeds a certain degree. These tubes eliminate the liability of the 5 passage of steam through the pipe D and into the mixing chamber E.

The relative proportions referred to may be varied within quite wide limits.

What is claimed is:—

- 10 1. A process for rendering crude oil residue available as a fuel which consists in first heating water to a temperature slightly below the thermal degree necessary for the formation of steam, feeding crude oil residue and the hot water to a common mixing chamber, mixing them to form an emulsion, and leading the emulsion to a burner.
- 15

2. A process of rendering Mexican flux or Mexican crude oil available as a fuel which consists in first heating water to a 20 temperature of from one hundred and fifty to two hundred and ten degrees Fahrenheit, feeding Mexican flux or crude oil and the hot water to a common point, mixing the same to form an emulsion, and leading the 25 emulsion to a burner.

In testimony whereof I affix my signature in presence of two witnesses.

OSCAR FALKENWALDE.

Witnesses:

Wm. TAYLOR, Jr.,  
JOHN T. FADDY.